

June 19, 1934.

F. C. T. DANIELS

1,963,403

LOCALLY HARDENED MOLYBDENUM STEEL ARTICLE OF MANUFACTURE

Filed Jan. 26, 1933

Fig. 1.



Fig. 2.



INVENTOR  
Fred C. T. Daniels  
By Green & McCallister  
His Attorneys

## UNITED STATES PATENT OFFICE

1,963,403

LOCALLY HARDENED MOLYBDENUM STEEL  
ARTICLE OF MANUFACTURE

Fred C. T. Daniels, Pittsburgh, Pa.

Application January 26, 1933, Serial No. 653,629

1 Claim. (Cl. 148—21)

My invention relates to the hardening of alloy steels and more specifically to the local surface hardening of cast or rolled molybdenum steels.

I am aware that local surface hardening has heretofore been practiced upon ordinary carbon steels such as those with a carbon content of about .32 to .65%, but that with such steels it is impossible to control the depth of penetration of the hardness, the uniformity thereof and the degree of hardness of the surface itself. I have found, for example, that the depth of hardness in such carbon steels varies at least from one-sixteenth of an inch to three-sixteenths of an inch under approximately the same heating conditions and varies in degree of hardness from 40 to 65 scleroscope.

I am also aware that it has been attempted with more or less success to surface harden steels in other ways. For example, it is known to case-carbonize or case-harden carbon steels or articles by impregnating the surfaces of initially low carbon steels after which the articles or the steels are quenched from the carbonizing heat or re-heated, quenched and drawn. Such treatment, however, alters the chemical composition of the surface to be hardened and, while it is capable of certain general localization, it is not possible to obtain true local surface hardening with any degree of accuracy or control.

In addition, such case-carbonization or case-hardening introduces considerable distortion into the pieces with the result that subsequent grinding or machining is required to restore true ness. Further than this, such case-carbonized or case-hardened articles require complete heating after machining and case carbonizing and then liquid quenching. In case-carbonizing also the case must of necessity follow the whole contour of the outer surface yielding as much hardness and consequent weakness at the base, both of which properties at that point being unnecessary and harmful. Such case-carbonized or hardened articles develop at most a hardness of only about 50 to 70 scleroscope, depending upon the size and other factors. For the same heating conditions the depth of hardening is uncontrollable and varies from  $\frac{1}{16}$ " to  $\frac{3}{16}$ ".

In what is known as the full hardened articles, steels or alloy steels are machined for finishing purposes on the hardened parts and then furnace heated to quenching temperature and then subjected to a liquid quench. In articles of the larger sizes particularly the hardness obtainable is very limited being not over about 40 to 60 55 scleroscope. This may be in part explained by

the fact that in the larger articles the mass of the article is so great or the variability of cross-section is so marked that drastic quenching is impossible.

In contradistinction to the foregoing, I have 60 obviated all the defects and disadvantages of such prior procedure and such accordingly constitutes one of the objects of my present invention.

Another object of my invention is to so correlate the composition of the steel and the hardening procedure that I obtain an article having an especially hard surface and in which the line of demarcation between the hardened and unhardened areas is so sharp that it does not extend in either direction as much as one one-hundredth 70 (1/100) of an inch.

A further object of my invention is the provision of local surface hardening for steels or articles of the kind hereinafter set forth wherein the line of demarcation between the hardened 75 and unhardened areas does not follow the crystal boundaries but takes a direct course on a straight line regardless of grain boundaries, therefore cutting through some grains.

An additional object of my invention is to so 80 locally surface harden molybdenum steel containing for example over about .2 up to about .5% molybdenum that the temperature at which the hardening may be carried out falls within a relatively wide and convenient range and further in 85 which the depth of hardening can be accurately controlled.

A still further object of my invention is a molybdenum steel article or piece having a hardened surface of predetermined and controllable depth 90 and having a hardness equivalent to about 90 to 100 scleroscope.

Other and further objects and advantages will either be pointed out hereinafter or will be understood by those skilled in this art.

By way of illustration I have shown in a comparative manner the effect and product of the present invention as applied in a manner consistent therewith and wherein:

Figure 1 represents a cross-section of an un-hardened molybdenum steel bar or article; and

Fig. 2 represents the bar or article of Fig. 1 after it has been hardened in accordance with the principles of the present invention.

In Figs. 1 and 2, the numeral 10 indicates the 105 unhardened portion of the molybdenum steel, bar or article to which the method of the present invention has not yet been applied and 11 represents the hardened portion after subjecting the bar or article 10 to my method of the present in- 110

- vention. The numeral 12 indicates the boundary line or line of demarcation between the unhardened area 10 and the hardened area 11. It will be understood that the figures are more or less diagrammatical and to that extent must be so considered merely as indicative. It will be noted further that the hardened area 11 is of much finer grain structure than unhardened area 10 but insofar as I am aware there has been no chemical change brought about by my method primarily due to the fact that I do not use any chemicals or hardening agents other than heat itself. Insofar as it is possible to show the same in a simple drawing it will be further observed that the boundary line or line of demarcation 12 is a sharp one so that the areas 10 and 11 do not appreciably cross this line and by suitable tests I have discovered that the line 12 is so sharp that the areas 10 and 11 do not overlap even to one one-hundredth of an inch. Moreover, by micro study I have discovered that this line 12 is not only of the sharpness indicated but it does not follow the crystal boundaries which would have the effect of rendering the line 12 of a more or less jagged or "saw-tooth" type, but on the contrary the line travels in a true straight line and thus crosses or intersects certain of the grains and boundaries with the degree of sharpness above pointed out.
- 30 In carrying out the present invention I either start with molybdenum steel containing from about .2 to .5% molybdenum or to available or satisfactory low carbon steels I add such an amount of molybdenum in suitable form at a suitable stage in the manufacture thereof as will produce in the finished steel about .2 to .5% molybdenum. In some cases I need merely remelt the steel and add the proper amount of molybdenum thereto, but in other cases where I am making up a batch of steel I add the molybdenum in any of the recognized stages of manufacture and in desired form such as ferro-molybdenum, elemental molybdenum and the like or equivalent.
- Having obtained the steel of the desired molybdenum content with or without other elements such as nickel, chromium, vanadium, etc. in small amounts to impart any desired physical properties to the steel or article when finished, I then carry out the local surface hardening in any selected one of the following ways according to the circumstances and conditions involved in any particular batch or article. The precise hardness in any given case varies somewhat with the percentage of carbon and the percentages of other elements in the steel.
- 60 One preferred way of carrying out the surface hardening is by means to a torch such as an oxy-acetylene welding torch which may have either one tip or two tips so that double width hardening may be simultaneously produced or so that (when the tips are arranged at angles to each other) I may harden simultaneously two surfaces, such as both sides of a gear or pinion tooth, at one time. Such torch is adjusted so that the flame is of a character which will make possible a rapid input of heat to the molybdenum steel article. Assuming a bar or article of the general nature illustrated in the drawings, I torch harden the surface thereof at the rate of about six inches per minute, that is, I so time the rate of movement or progress of the torch that six inches of steel are hardened per minute. While this hardening is being carried out the article is immersed in circulating cold water to a point just below the depth of hardness required. In

addition, the torch is followed by a stream of cooling or quenching water which proceeds directly behind the torch.

I find that on carrying out such hardening on such material particularly when under the general conditions above noted I obtain a very unexpected type and degree of hardness and one which is entirely controllable as to depth as well as to a hardness which is absolutely uniform throughout the hardened area. A further and important result and advantage is that instead of being forced to carry out the hardening at a specific temperature without appreciable variation thereabove or therebelow I find that I no longer need to maintain such close and commercially impractical control over the temperature, but that uniform hardness can be obtained merely by maintaining the temperature of the hardening heat within the general limits of about 1250° and 1700° F. Not only this, but I find that the depth of hardening is proportional to the time of application of the hardening heat—the longer the time, the greater the depth, other factors being the same,—so that by subjecting the material or article to the hardening heat within the temperature range stated for a predetermined time, I may obtain the hereinabove pointed out results.

Furthermore, the line of demarcation between the hardened and unhardened areas is exceedingly distinct and much sharper than anything heretofore obtained by any method of hardening insofar as I am aware. As above indicated the line of demarcation is so sharp that the hardened and unhardened areas do not overlap even to the extent of one one-hundredth of an inch insofar as I am able to determine by available tests. This sharp line furthermore does not follow the crystal boundaries but proceeds in a true straight line irrespective of grain boundaries.

In the particular sample illustrated in the drawing I have obtained by the present invention a hardened area having a hardness of 90 to 100 scleroscope. In some larger articles where the rate of cooling is appreciably slower I have obtained a hardness of the order of 80 to 90 scleroscope and in some instances I find that the minimum hardness is about 70 to 80 scleroscope under less favorable conditions due to the nature of the article or for other reasons understood by those skilled in this art. I have made many tests and find that the sharp line of demarcation is not a line of weakness. By no test have I been able to cause a partition at this line of juncture. I have even pounded the article while cold under a steam hammer until it was reduced one-eighth in thickness without damaging the hardened surface in any way, and without causing it to spall or flake off, indicating a perfect bond between the hardened and unhardened areas. The samples are file-hard and will frequently scratch glass.

As I have stated above, the molybdenum content may vary from about .2% to about .5%, the intention being that these percentages are typical rather than limitative, and the remaining elements of the steels may also vary as will be understood. In general, the sulphur, phosphorus, manganese and silicon are within the usual limits found in steel making practice, that is, are within amounts classified as impurities and are so small as to have no appreciable influencing effect on the alloy.

The following ranges of elements approximate-

ly define successful practice according to the present invention:

|    |                               | Percent  |
|----|-------------------------------|----------|
| 5  | Silicon                       | .10-.40  |
|    | Sulphur                       | .01-.06  |
|    | Phosphorus                    | .01-.08  |
|    | Manganese                     | .30-.150 |
|    | Carbon                        | .30-.125 |
| 10 | Molybdenum and, when present: | .10-.75  |
|    | Nickel                        | .25-.150 |
|    | Chromium                      | .10-.110 |
|    | Vanadium                      | .08-.25  |

15 The following Table I gives a number of open hearth heats illustrative of steels giving the above results when subjected to the hardening process described:

| 20 | Si  | S    | P    | Mn   | C    | Ni    | Cr    | Mo  |
|----|-----|------|------|------|------|-------|-------|-----|
|    | .32 | .028 | .033 | 1.08 | .48  | Trace | Trace | .27 |
|    | .40 | .022 | .037 | 1.00 | 1.25 | 1.41  | 1.08  | .29 |
|    | .40 | .020 | .040 | 1.14 | .41  | .37   | .28   | .39 |
|    | .30 | .035 | .031 | .89  | .85  | 1.58  | .84   | .27 |
| 25 | .33 | .018 | .032 | 1.25 | .80  | 1.50  | .46   | .35 |
|    | .34 | .017 | .033 | 1.20 | .76  | 1.38  | .53   | .37 |
|    | .31 | .020 | .040 | 1.10 | .46  | Trace | Trace | .30 |
|    | .32 | .031 | .038 | .82  | 1.14 | 1.37  | 1.09  | .25 |
|    | .30 | .024 | .037 | .87  | .83  | 1.38  | .95   | .24 |
|    | .25 | .018 | .037 | 1.34 | .80  | 1.45  | .35   | .25 |
|    | .31 | .016 | .034 | .95  | .44  | Trace | Trace | .22 |
| 30 | .25 | .030 | .027 | 1.10 | .63  | Trace | Trace | .34 |
|    | .41 | .027 | .028 | .87  | .49  | 1.51  | 1.12  | .22 |
|    | .30 | .023 | .033 | 1.02 | .80  | 1.46  | 1.05  | .33 |
|    | .38 | .020 | .034 | 1.21 | .48  | 1.46  | .07   | .27 |
|    | .26 | .030 | .034 | .52  | .44  | 1.55  | .90   | .26 |
|    | .38 | .024 | .043 | 1.42 | 1.30 | .73   | 1.00  | .40 |
|    | .38 | .021 | .040 | .80  | .91  | 1.48  | 1.00  | .27 |
|    | .36 | .024 | .035 | .88  | .47  | 1.60  | .96   | .22 |
| 35 | .31 | .024 | .029 | .75  | .47  | 1.63  | 1.02  | .27 |
|    | .28 | .014 | .036 | .95  | 1.23 | 1.62  | .83   | .22 |

The following Table II represents a number of other steels hardened by the foregoing process other than the above open hearth heats:

| 40 | Si  | S    | P    | Mn  | C   | Ni   | Cr  | Mo  | Va  |
|----|-----|------|------|-----|-----|------|-----|-----|-----|
|    | .24 | .026 | .030 | .67 | .30 | 1.75 | .72 | .40 | .09 |
|    | .26 | .030 | .030 | .62 | .47 | 1.35 | .77 | .23 | .17 |
| 45 | .24 | .025 | .028 | .65 | .54 | 1.35 | .72 | .23 |     |

The present invention is not limited, however, to gear or pinion teeth but applies equally well to pug mill knives, pulverizer hammers, shuffle board weights, crusher rings, pinions, gears, guides, couplings, bevel gears, shovel points, punches, etc.

By my invention I do not alter the chemical

composition of the hardened surface to any degree whatsoever, but the hardness is obtained by rapid local heating and rapid cooling as above set forth. I can also localize the hardness to very small zones or areas such as small saw-tooth corrugations or special cutting shapes on corrugated rolls. Nor does the present invention affect the base or unhardened metal in any manner but leaves the same in its original strong condition. I need only harden and quench the particular area to be hardened. Unusually good wearing surfaces are thus obtained.

I may, if desired, carry out the heating by a suitably constructed and arranged electrical apparatus such as one of the resistance or conduction type. The precise form of such apparatus forms, per se, no part of the present invention. The type of heat seems to have no real influence upon the results obtainable by the present invention and it is accordingly within the scope of my invention to utilize heat generated electrically in suitable manner.

What I claim as new and desire to secure by Letters Patent is:

A substantially chromium-free cast molybdenum steel article of manufacture composed of an alloy containing:

| About percent |          |     |
|---------------|----------|-----|
| Silicon       | .10-.40  | 105 |
| Sulphur       | .01-.06  |     |
| Phosphorus    | .01-.08  |     |
| Manganese     | .30-.150 |     |
| Carbon        | .30-.125 |     |
| Molybdenum    | .10-.75  | 110 |

and the balance substantially all iron, said article of manufacture being characterized by having a hardened surface produced by rapidly heating the same by subjection to a flame to 1250-1700° F. and then quenching; and further characterized by the fact that the flame hardened portion has a finer grain structure than the unhardened portion, the chemical composition of the hardened portion is the same as the unhardened portion, the hardened and unhardened portions are relatively sharply delimited from one another, the depth of hardness is fully under control and is directly proportional to the time during which the hardening heat is applied, and a uniform hardness of 70-100 scleroscope is readily attained.

FRED C. T. DANIELS.

55

60

65

70

75

80

85

95

100

105

110

115

120

125

130

135

140

145

150